# EUROPEAN PATENT SPECIFICATION

(11) **EP 0 347 127 B1**
(45) Date of publication and mention of the grant of the patent: **25.11.1992**
(21) Application number: 89305873.5
(22) Date of filing: 09.06.1989
(51) Int. Cl.: C10M 159/18, C10M 133/52

(54) **Method for preparing salts of polyolefinic substituted dicarboxylic acids in oleaginous mixtures of reduced viscosity**
Verfahren zur Herstellung von Salzen aus polyolefin-substituierten Dicarbonsäuren in Ölgemischen mit schwacher Viskosität
Procédé de préparation de sels d'acides dicarboxyliques substitués par des polyoléfines dans des mélanges oléagineux à faible viscosité

(30) Priority: 16.06.1988 US 207611
(43) Date of publication of application: 20.12.1989
(73) Proprietor: EXXON CHEMICAL PATENTS INC., Florham Park New Jersey 07932 (US)
(72) Inventor: Colcord, Laura Jean, Maplewood New Jersey 07040 (US); Emert, Jacob, Brooklyn New York 11218 (US); Waddoups, Malcolm, Westfield New Jersey 07090 (US); Lundberg, Robert Dean, Bridgewater New Jersey 08807 (US)
(74) Representative: Northover, Robert Frank

(56) References cited:
- FR-A- 1 422 401
- US-A- 3 306 908

## Description

This invention is directed generally to a process for preparing copper salts of polyolefinic substituted dicarboxylic acids and more particularly to a process for preparing oleaginous mixtures of such copper salts having reduced viscosity and decreased viscosity growth. The method involves the steps of providing a copper salt of a polyolefinic substituted dicarboxylic acid, and thereafter contracting the product of the first step with a specific class of amines.

There are several methods for preparing the Group I-B and II-B metal salts of polyolefinic substituted dicarboxylic acids.

US-A-4552677 describes a process wherein a copper compound such as cupric acetate hydrate, basic cupric acetate, cuprous carbonate, basic cupric carbonate, and cuprous or cupric hydroxide is introduced into a reaction vessel containing a hydrocarbyl substituted succinic anhydride derivative. A variety of acidic, neutral and basic copper salts are shown as products. The hydrocarbyl group has a maximum of 35 carbon atoms.

Similarly US-A-3271310 shows the production of a similar selection of salts, including Group I-B metal salts, using analogous technology.

US-A-3574101 discloses the preparation of oil-soluble carboxylic acid acylating agents by reacting a high molecular weight mono- or polycarboxylic acid with a sulfonating agent. The resulting acylating agents are disclosed to be useful as intermediates in the preparation of metal salts, and the metal salts and the acylating agents are disclosed to be useful additives for lubricants and fuels and as intermediates for preparation of other Lubricant and fuel additives, particularly high molecular weight oil-soluble acylated nitrogen compositions and esters. Such nitrogen compositions are exemplified by reaction of a tetraethylene pentamine with the sodium salt of a polyisobutylene succinic anhydride-chlorosulfonic acid product.

US-A-3652616 relates to additives for fuels and lubricants prepared by reacting a hydrocarbon-substituted succinic anhydride and an alkylene polyamine to form a material which is then reacted; with one of a recited class of metallic materials including metal salts of carboxylic acids, metal thiocyanates, metal acid complexes (e.g., acids having cyanate, chloride, or thiocyanate moieties) and metal oxides or sulfides.

GB-A-1,054,280 describes amide and imide derivatives of metal salts of substituted succinic acids in which the substituent is a hydrocarbon having at least 50 aliphatic carbon atom. The metals employed are the alkali metals, alkaline earth metals, lead, cadmium and zinc.

The present invention provides a process for producing an oleaginous solution containing copper salts of olefinic dicarboxylic acids having reduced viscosity comprising the steps of:
(a) providing a copper salt of a polyolefinic substituted dicarboxylic acid material, said polyolefinic substituent being derived from an olefin polymer of a C₂ to C₁₀ monoolefin having a number average molecular weight greater than 600, and said dicarboxylic acid moiety being derived from a C₄ to C₁₀ monounsaturated dicarboxylic acid material; and
(b) reacting or complexing at least a portion of the product of step (a) in a liquid reaction solvent with an amine selected from aliphatic and cycloaliphatic amines containing from 1 to 4 nitrogen atoms per molecule, said amine having at least one primary or secondary nitrogen atom per molecule.

The process uses inexpensive amine and copper bearing reactants. The polyolefinic substituted dicarboxylic acid copper salts can be obtained in a variety of ways.

The resulting oleaginous compositions have been found to have a significantly reduced viscosity, and also to undergo substantially less viscosity growth during storage. They are much easier to handle and use than those obtained in the absence of such amine-treatment step, as in EP-A-273626.

The compositions have a variety of utilities as, for instance, compatibilising agents or dispersants in lubricating oil formulations.

### Description of preferred embodiments

### Copper salts of polyolefinic substituted dicarboxylic acids

The copper salts of polyolefinic substituted dicarboxylic acids preferred for treatment in step (b) may be derived by reacting an organic or inorganic copper compound with long chain polyolefinic substituted dicarboxylic acid materials, i.e. acid anhydride or ester, in turn derived from alpha or beta unsaturated C₄₋₁₀ dicarboxylic acids (e.g. itaconic acid, maleic acid, maleic anhydride, chloromaleic acid, chloromaleic anhydride, dimethyl fumarate and mixtures thereof.)

Preferred olefin polymers which may be reacted with the above unsaturated acid materials contain a major molar amount of C₂₋₁₀ monoolefin, e.g. C₂₋₅ monoolefin. Examples are ethylene, propylene, butylene, isobutylene, pentene, octene-1, and styrene. The polymers may be homopolymers such as polyisobutylene or copolymers of two or more such olefins. These include copolymers of: ethylene and propylene; butylene and isobutylene; propylene and isobutylene; etc. Other copolymers include those in which a minor molar amount of the copolymer monomers, e.g., 1 to 10 mole percent, is a C₄ to C₁₈ diolefin, e.g., copolymers of isobutylene and butadiene; or copolymers of ethylene, propylene and 1,4-hexadiene, 5-ethylidene- 2-norbonene; etc.

In some cases, the olefin polymer may be completely saturated, for example, an ethylene-propylene copolymer made by a Ziegler-Natta synthesis using hydrogen as a moderator to control molecular weight.

The olefin polymers have number average molecular weights (Mₙ) above about 600. Particularly useful olefin polymers have number average molecular weights within the range of about 900 and about 5,000 with approximately one double bond per polymer chain. An especially suitable starting material is polyisobutylene. The number average molecular weight for such polymers can be determined by several known techniques. A convenient method for such determination is by gel permeation chromatography (GPC) which additionally provides molecular weight distribution information (see W. W. Yua, J. J. Kirkland and D. D. Bly, "Modern Size Exclusion Liquid Chromatography," John Wiley and Sons, New York, 1979).

Processes for reacting the olefin polymer with the C₄₋₁₀ unsaturated dicarboxylic acid, anhydride or ester are known in the art. For example, the olefin polymer and the dicarboxylic acid material may be simply heated together as disclosed in US-A-3361673 and US-A-3401118 to cause a thermal "ene" reaction to take place. Or, the olefin polymer can be first halogenated, for example, chlorinated or brominated to about 1 to 8, preferably 3 to 7 weight percent chlorine, or bromine, based on the weight of polymer, by passing the chlorine or bromine through the polyolefin at a temperature of 100° to 250°, e.g., 140° to 225°C for about 0.5 to 10, e.g., 3 to 8 hours. Processes of this general type are taught in US-A-3087436; US-A-3172892; US-A-3272746 and others.

Alternatively, the olefin polymer, and the unsaturated acid material are mixed and heated while adding chlorine to the hot material. Processes of this type are disclosed in US-A-3215707; US-A-3231587; US-A-3912764; US-A-4110349; US-A-4234435; and in GB-A-1440219.

By the use of halogen, about 65 to 95 weight percent of the polyolefin will normally react with the dicarboxylic acid material. Thermal reactions, those carried out without the use of halogen or a catalyst, cause only about 50 to 75 weight percent of the polyisobutylene to react. Chlorination obviously helps to increase the reactivity.

The copper salt can comprise an acid or neutral salt of the selected polyolefinic dicarboxylic acid material. By "acid salt" is meant a material which is a half-salt of the dicarboxylic acid. By "neutral salt" is meant a material in which both carboxy groups of the dicarboxylic acid material form copper salts.

Preferred polyolefinic substituted dicarboxylic acids are polyisobutenyl succinic acid, polybutenyl succinic acid, and the anhydrides thereof.

Especially preferred are copper salts of polyisobutenyl succinic acid and polyisobutenyl succinic anhydride wherein the polyisobutenyl group is derived from a polymer having a number average molecular weight of from about 900 to about 3000.

The copper salts of such polyolefinic substituted dicarboxylic acids can be prepared by any convenient method. For example, the selected polyolefinic substituted dicarboxylic acid or anhydride can be reacted with an inorganic compound containing copper (e.g., The metal oxide, carbonate, hydroxide, and the like) for a time and under conditions sufficient to form the desired metal salt of the polyolefinic substituted dicarboxylic acid (e.g., at 100°C for 8 hours). The reaction medium can then be stripped with an inert gas (e.g. N₂ gas stripping for 3 hours at 135°C) to remove the water of reaction. Alternately, the polyolefinic substituted dicarboxylic acid or anhydride can be reacted with an organic compound of the metal (e.g., a metal alkanoate salt, such as the acetate or propionate), again followed by stripping.

A preferred method is disclosed in EP-A-273626 wherein the copper salts are prepared by reaction of an inorganic compound of the copper (e.g., The oxide, carbonate, hydroxide, and the like) with the polyolefinic substituted dicarboxylic acid or anhydride in the presence of a short chain alkanoic acid (e.g. acetic or propionic acid). The reaction is typically carried out in a liquid reaction solvent comprising a hydrocarbon oil (such as a mineral oil, synthetic lubricating oil and the like) and will be typically conducted at a temperature in the range of from about 70 to 150^C, followed by stripping with unreactive gas, such a nitrogen, to remove various light materials (such as unreacted alkanoic acid) and then filtered to remove any insolubles, such as unreacted copper-containing starting materials and by-products. Alternatively, the filtering at this stage can be deferred until completion of the amine-contacting step, which will now be described below.

In the above processes, water will be generally introduced into the reaction medium if the selected polyolefinic substituted dicarboxylic acid material comprises the anhydride, to facilitate reaction of the desired dicarboxylic acid groups.

### Amine Reactants

The metal salt product obtained as above can also contain quantities of unreacted polyolefin substituted dicarboxylic acid or corresponding anhydride. Where present, the concentration of unreacted polyolefin substituted dicarboxylic acid or corresponding anhydride will generally range from about 1 to 20 wt%, more typically from about 5 to 15 wt%. It has been found that this metal salt product is a very viscous component of lubricating oils and that its viscosity increases upon storage, most likely because of aggregation of its contained ionic species. This leads to difficulties in manufacturing, handling and using the metal salt product, e.g., in lubricating oils as an antioxidant. It has been found that these problems can be minimized by contracting the metal salt product with certain amines. This contacting treatment both decreases the initial viscosity of the product and reduces the rate of viscosity growth.

In this second step of the process of this invention, the copper salt product is contacted with at least one member of a certain class of amine treatment compounds under conditions sufficient for reaction (or complexation) of the amine with at least a portion of the polyolefin substituted dicarboxylic acid copper salt product, that is, the product mixture containing the polyolefinic substituted dicarboxylic acid groups previously reacted with the copper, and unreacted quantities of the polyolefinic substitued dicarboxylic acid material. The amine treatment compound, therefore, should be one which is reactive with the carboxylic acid or anhydride groups of the dicarboxylic acid material, but it should also not interact with the copper salt in such a way as to form an insoluble, copper-containing precipitate. Furthermore, it is preferred, although not required, that the amine compound be one which has a convenient boiling point to allow any excess amine to be easily stripped out from the amine contacting mixture.

It has been surprisingly found that alkylene polyamines having greater than about 5 nitrogen atoms, which are typically employed in the manufacture of lubricating oil nitrogen-containing dispersant additives, form undesirable side-reactions with the metal component in the additive to be treated, as will be further discussed below. For example, poly(ethyleneamine) compounds averaging from above about 5 to 7 nitrogen atoms per molecule, which are available commercially under trade names such as "Polyamine H", "Polyamine 400", and "Dow Polyamine E-100", should not be employed as amine treatment compounds in this invention since they have been found to cause precipitation of the copper salts from the copper salt products.

Useful amine treatment compounds for this invention comprise at least one member selected from the group consisting of aliphatic and cycloaliphatic amines containing from 1 to 4 nitrogen atoms per molecule, wherein at least one of the nitrogen atoms is primary or secondary. Generally, the amine compound will contain up to about 25 carbon atoms, and preferably up to about 15 carbon atoms, per molecule.

Therefore, useful amines for this invention include linear and branched polyethylene or polypropylene amines containing up to 4 nitrogens per molecule. The nitrogen atoms may be secondary or primary, and preferably the amine reactant contains at least one primary amine. Most preferably, the amine compound contains from 1 to 2 primary amine groups.

These amines may be hydrocarbyl amines or may be hydrocarbyl amines including other groups, e.g, hydroxy groups, alkoxy groups, amide groups, nitriles, imidazoline groups, and the like. Hydroxy amines with 1 to 3 hydroxy groups, preferably 1 hydroxy group, are particularly useful. Preferred amines are aliphatic saturated amines, including those of the general formulas:
wherein R, R′, R˝ and R˝′ are independently selected from the group consisting of hydrogen; C₁ to C₂₅ straight or branched chain alkyl radicals; and C₁ to C₁₂ alkoxy C₂ to C₆ alkylene radicals; and wherein R˝′, can additionally comprise a moiety of the formula:
wherein R′ is as defined above, and wherein each s and s′ can be the same or a different number of from 2 to 6, preferably 2 to 4; and t and t′ can be the same or different and are each numbers of typically from 0 to 2, preferably 1, with the proviso that the amine contains not greater than 4 nitrogen atoms. To assure a facile reaction it is preferred that R, R′, R˝, R˝′, (s), (s′), (t) and (t′) be selected in a manner sufficient to provide the compounds of formulas Ia and Ib with typically at least one primary amine group, preferably two primary amine groups.

Non-limiting examples of suitable amine compounds include: 1,2 -diaminoethane; 1,3-diaminopropane; 1,4-diaminobutane: 1,6-diaminohexane; polyethylene amines such as diethylene triamine and triethylene tetramine; 1,2-propylene diamine; polypropylene amines such as di-(1,2-propylene)triamine and di-(1,3-propylene) triamine; N,N-dimethyl-1,3-diaminopropane; N,N-di-(2-aminoethyl) ethylene diamine; N,N-di(2-hydroxyethyl)-1,3-propylene diamine; 2-propyldodecylamine; N-dodecyl-1,3-propylene diamine; diisopropanol amine; diethanol amine; amino morpholines such as N-(3-aminopropyl) morpholine; and mixtures thereof.

Other useful amine compounds include: alicyclic diamines such as 1,4-di(aminomethyl) cyclohexane, and heterocyclic nitrogen compounds such as imidazolines, and N-aminoalkyl piperazines of the general formula (II):
wherein p₁ and p₂ are the same or different and are each integers of from 1 to 4, n₁ and n₃ are the same or different and are each integers of from 0 to 3, and n₂ is 0 or 1, with the proviso that the sum of n₁, n₂ and n₃ is not greater than 3. Non-limiting examples of such amines include N-(2-aminoethyl) piperazine.

Commercial mixtures of amine compounds may advantageously be used, provided they contain an average of not greater than about 4 nitrogen atoms per molecule. For example, one process for preparing alkylene amines involves the reaction of an alkylene dihalide (such as ethylene dichloride or propylene dichloride) with ammonia, which results in a complex mixture of alkylene amines wherein pairs of nitrogens are joined by alkylene groups, forming such compounds as diethylene triamine, triethylenetetramine and corresponding piperazines.

Useful amines also include polyoxyalkylene polyamines such as those of the formulae:
where m has a value of 1 to 2; and
where "n" has a value of 1 to 2, and R is a substituted saturated hydrocarbon radical of from 1 to 3 carbon atoms, wherein the number of substituents on the R group is represented by the value of "a", which is a number from 1 to 3. The alkylene groups in either formula (III) or (IV) may be straight or branched chain and contain from 2 to 4 carbon atoms.

The amine treatment compound and metal salt product are contacted in the presence of a liquid medium which can comprise an inert diluent or solvent for the reactants. Generally useful are hydrocarbon solvents, such as mineral oils, synthetic lubricating oils, and the like. For example, the solvent employed in the preparation of the metal salt product can be passed to the amine contacting step.

The amine can be readily reacted or complexed with the dicarboxylic acid copper salt material, e.g., the copper salt product of polyalkenyl substituted succinic anhydride, by contacting the selected amine compound with the copper salt product for a time and under conditions sufficient to react (or complex) the amine with at least a portion of the polyolefinic substituted dicarboxylic acid metal salt product. Generally, the amine and the copper salt product will be contacted with stirring at a temperature of from about 100 to 150°C., preferably 110 to 135°C., generally for 0.3 to 10, e.g., 30 min. to 3 hours. The contacting is preferably conducted in an inert atmosphere (e.g., under N₂). Treatment ratios of the dicarboxylic acid metal salt product to equivalents of amine can vary considerably, depending upon the reactants and type of bonds formed. The selected amine should be introduced in amount sufficient to provide an excess of reactive primary or secondary amine above that amount of reactive primary or secondary amine required for reaction with the equivalents of free polyolefinic substituted dicarboxylic acid or anhydride and for complexation with the copper in the copper salt product. Generally, the selected amine compound is introduced in amount sufficient to provide form about 1 to 10, preferably about 1.5 to 5, equivalents of reactive primary or secondary amine per mole of dicarboxylic acid moiety content of the polyolefinic substituted dicarboxylic acid or anhydride copper salt product so treated. After the desired contacting time, the contacting mixture is preferably stripped (e.g., with N₂ or other substantially insert gas) at elevated temperature (e.g., from about 120 to 150°C) to remove water of reaction and remaining amine which has not reacted or complexed with the copper salt product.

After stripping unreacted amine and water from the reaction mixture, the product is filtered to remove process sediment and unconverted metal reactants (if the latter have not been sufficiently removed in filtering of the metal salt product charged to the amine reaction step of the process). The resulting solution will be generally characterized by a kinematic viscosity of from about 200 to 1400.10⁻⁶m^{2s-1} (at 100°C). The products prepared by the process of this invention will generally comprise form about 20 to 60 wt%, more typically from about 20 to 45wt%, of the copper salt of the polyolefinic substituted dicarboxylic acid material (both amine complexed and uncomplexed), from about 1 to 20 wt%, more typically from about 2 to 10 wt%, of the non-copper-containing reaction product formed by reaction of the amine and the polyolefinic substituted dicarboxylic acid material, and from about 25 to 80 wt%, more typically from about 40 to 60 wt%, of a lubricating oil (e.g., a lubricating oil of the type conventionally used in crankcase lubricating oils as described below).

The lubricating oil additives prepared by the process of this invention, as described above, have advantageously improved viscosity properties and are useful as lubricating oil additives, e.g. as antioxidants, in internal combustion crankcase lubricating oils (e.g., automotive engines, which are fueled by gasoline, methanol, diesel and other conventional fuels). Accordingly, the additive can be used by incorporation and dissolution into an oleaginous material such as fuels and lubricating oils. When the additive mixtures of this invention are used in normally liquid petroleum fuels such as middle distillates boiling from about 65° to 430°C, including kerosene, diesel fuels, home heating fuel oil, jet fuels, etc., a concentration of the additives in the fuel in the range of typically from about 0.001 to about 0.5, and preferably 0.005 to about 0.15 weight percent, based on the total weight of the composition, will usually be employed.

The additive mixtures of the present invention find their primary utility in lubricating oil compositions which employ a base oil in which the additive is dissolved or dispersed. Such base oils may be natural or synthetic. Base oils suitable for use in preparing the lubricating oil compositions of the present invention include those conventionally employed as crankcase lubricating oils for spark-ignited and compression-ignited internal combustion engines, such as automobile and truck engines, marine and railroad diesel engines, and the like. Advantageous results are also achieved by employing the additives of the present invention in base oils conventionally employed in and/or adapted for use as power transmitting fluids such as automatic transmission fluids, tractor fluids, universal tractor fluids and hydraulic fluids, heavy duty hydraulic fluids, power steering fluids and the like. Gear lubricants, industrial oils, pump oils and other lubricating oil compositions can also benefit from the incorporation therein of the additives of the present invention.

These lubricating oil formulations conventionally contain several different types of additives that will supply the characteristics that are required in the formulations. Among these types of additives are included viscosity index improvers (e.g., ethylene-propylene copolymer VI improvers, dispersant-viscosity improver polymers, and the like), supplemental antioxidants, corrosion inhibitors, detergents (e.g., neutral or basic (including overbased) alkali and alkaline earth metal salts of alkyl phenates, sulfurized alkyl phenates, alkylsulfonic acids, etc.), dispersants (e.g., high molecular weight ashless nitrogen- and ester-containing dispersants and the borated derivates thereof), pour point depressants, antiwear agents (e.g., zinc dialkyldithiophosphates), friction modifiers (e.g., glycerol oleates), etc. Suitable such other additives for use in combination with the additives of the present invention are disclosed in EP-A-273626, EP-A-275658, and EP-A-271362.

This invention will be further understood by reference to the following examples, wherein all parts are parts by weight, unless otherwise noted. In the Examples, the term "Sap. No." refers to the saponification number of the indicated materials, in units of mg KOH/G., as determined by ASTM Method D94.

### Examples

### Example 1

(a) About 3830 g. (3.8 mole) of a polyisobutenyl succinic anhydride (Sap. No. 111) derived from a 950 M̅ₙ polyisobutylene is charged to a stirred reaction flask equipped with a reflux condenser, and 850 g. of cupric acetate monohydrate (31.3 wt% Cu), 3020 g. of diluent oil solvent (150N) and 175 g. of water are added. The reaction mass is heated to 110°C, after which it is soaked for one hour and then stripped for one hour with dry N₂ gas. Subsequently, 85 g. of water are added to the mixture, and the soaking and stripping steps are repeated. Four more water additions (of between 70 and 100 g. of water each), with the accompanying soaking and stripping steps, are carried out. The reaction mixture is then stripped with dry N₂ for 3 hours and filtered to remove any unreacted solids or solid by-products. The filtrate analyzes for 2.85 wt.% copper.
(b) To 100 g. of the product of step (a) is added 1.6 grams of diethylenetriamine (containing 38 wt.% nitrogen and having 3 nitrogen atoms per molecule) at a temperature of about 120°C. After the amine addition, the mixture is allowed to react for 30 minutes. Thereafter, unreacted amine and the water of reaction is removed from the reaction medium using a 2-hr. dry N₂ strip at 120°C. The resulting liquid is then filtered to remove process sediment. The resulting filtrate analyzes for 2.84 wt.% copper.

### Example 2

(a) About 100 g. of a polyisobutenyl succinic anhydride (Sap. No. 106.9) derived from a 950 number average molecular weight polyisobutylene polymer, is charged to a reaction flask, and 67.6 g. of diluent oil solvent 150N, 5 g. of water, and 20.9 g. of cupric acetate monohydrate are added. The reactants are heated to 110°C, and soaked and stripped as described in Example 1. Subsequently, three 1-g. additions of water, followed by soaking and stripping steps are carried out. The reaction mixture is then stripped with dry N₂ for 4 hours at 135°C. This intermediate product analyzes for 3.34 wt% copper.
(b) The reaction mass is then cooled to 120°C, and 2.8 g. of diethylenetriamine are added. The reaction mixture is allowed to react for 30 minutes. Unreacted amine and the water of reaction are removed using a 2-hour strip with dry N₂ gas. The resulting product is then filtered, and the filtrate is found to contain 3.3 wt% copper and 0.67 wt% nitrogen.

### Example 3

The procedure of Example 2 is repeated, except that the initial water charge is increased to 8.75 g. and after charging the raw materials the reaction mixture is heated to 110°C and held at that temperature for 6 hours. Then the reaction mixture is stripped with dry N₂ gas for 2 hours at 135°C. The amine treatment is carried out as in Example 2(b) above. The product is found to contain 3.3 wt % copper.

The products of the first and second stages in each of examples 1 through 3 are tested to determine their initial viscosities. Samples of each material are stored for from 1 to 4 weeks at either 25°C or 54°C to determine the rate of viscosity growth over this term. The data thereby obtained are summarized in Table I below.

As the above data show, the products of this invention in examples 1(b), 2(b), and 3(b) are characterized by initial viscosities which were considerably reduced over those of examples 1(a), 2(a), and 3(a), even though additional amine reacted with the products of the step (a) mixtures would have been expected to enhance the viscosity of these materials by virtue of the addition thereto of the amine reactant. Further, the products of this invention in examples 1(b), 2(b) and 3(b) showed much greater viscosity stability during storage, both at room temperature and at elevated temperature (54°C).

### Comparative Example 4

100 g. of the product as prepared in Example 1 (a) are charged to a stirred reaction flask, together with 2.5 g. of a polyethylene polyamine bottoms product (avg. approximately 6.5 nitrogen atoms and 11 carbon atoms per molecule). The mixture is heated to 120°C. An orange-brown precipitate forms, and continues to form until the original color of the metal succinate is no longer evident, thereby indicating that copper was removed from the additive solution due to side reactions with the charged alkylene polyamine.

### Example 5

(a) About 140 g. of a polyisobutenyl succinic anhydride (Sap. No. 69) derived from a 1300 number average molecular weight polyisobutylene polymer, is charged to a stirred reaction flask, and 56.9 g of additional diluent oil solvent 150N, 8.75 g. of water, and 18.1 g. of cupric acetate monohydrate are added. The reactants are heated to 110°C for 6 hours. Then, the reaction mixture is stripped with dry N₂ gas for 2 hours at 135°C.
(b) The reaction mass is then cooled to 120°C, and 3.0 g. of hexylamine are added. The reaction mixture is allowed to react for 60 minutes. Unreacted amine and the water of reaction are removed using a 2-hour strip with dry N₂ gas. The resulting product is then filtered, and the filtrate is found to contain 2.7 wt% copper and 0.2 wt% nitrogen.

### Example 6

(a) About 200 g. of a polyisobutenyl succinic anhydride (Sap. No. 43) derived from a 2200 number average molecular weight polyisobutylene polymer, is charged to a stirred reaction flask, and 66.1 g. of additional diluent oil solvent 150N, 10 g. of water, and 17 g. of cupric acetate monohydrate are added. The reactants are heated to 110°C for 6 hours. Then, the reaction mixture is stripped with dry N₂ gas for 2 hours at 135°C. The resulting product is then filtered, and the filtrate is found to have a kinematic viscosity of 1500 10⁻⁶m²⁻s⁻¹ (at 100°C) and to contain 1.59 wt% copper.
(b) The reaction mass is then cooled to 120°C, and 1.4 g. of dimethylaminopropyl amine are added. The reaction mixture is allowed to react for 30 minutes. Unreacted amine and the water of reaction are removed using a 2-hour strip with dry N₂ gas. The resulting product is then filtered, and the filtrate is found to contain 1.5 wt% copper and 0.27 wt% nitrogen and is found to have a kinematic viscosity of 1310 10⁻⁶ m²s⁻¹ (at 100°C).

### Example 7

About 80 g. of the product of Example 1 (a) are charged to a stirred reaction flask, along with 1.66 g. of dimethylaminopropyl amine. The reaction mixture is heated to 120°C and held at that temperature for 30 minutes. Then the reaction mixture is stripped with dry N₂ as for 2 hours. The resulting product is then filtered, and the filtrate is found to have a kinematic viscosity of 580 cSt (at 100°C) and to contain 2.62 wt% copper.

## Claims

1. A process for producing an oleaginous solution containing copper salts of polyolefinic dicarboxylic acids having reduced viscosity comprising the steps of:
(a) providing a copper salt of a polyolefinic substituted dicarboxylic acid material, said polyolefinic substituent being derived from an olefin polymer of a C₂ to C₁₀ monoolefin having a number average molecular weight greater than 600, and said dicarboxylic acid moiety being derived from a C₄ to C₁₀ monounsaturated dicarboxylic acid material; and
(b) a reacting or complexing at least a portion of the product of step (a) in a liquid reaction solvent with an amine selected from aliphatic and cycloaliphatic amines containing from 1 to 4 nitrogen atoms per molecule, said amine having at least one primary or secondary nitrogen atom per molecule.

2. A process according to claim 1 wherein said monounsaturated acid material comprises at least one member selected from maleic acid, maleic anhydride, itaconic acid, chloromaleic acid, chloromaleic anhydride, and dimethyl fumarate.

3. A process according to claim 1 or claim 2 wherein the polyolefinic substituent comprises polyisobutylene, polybutylene or mixtures thereof.

4. A process according to any preceding claim wherein the polyolefinic substituent is derived from a polymer having a number average molecular weight of 900 to 3000.

5. A process according to claim 4 wherein the polyolefinic substituted dicarboxylic acid material is selected from polyisobutenyl or polybutenyl succinic acid or anhydride.

6. A process according to any preceding claim wherein the amine comprises at least one aliphatic saturated amine of the general formulae: wherein R, R′, R˝ and R˝′ are independently selected from hydrogen, C₁₋₂₅ straight or branched chain alkyl, C₁₋₁₂ alkoxy, and C₂₋₆ alkylene, and wherein R˝′ can additionally comprise a moiety of the formula: wherein R′ is as defined above, and wherein each of s and s′ can be the same or a different number from 2 to 6, and t and t′ can be the same or a different number from 0 to 2, with the proviso that the amine contains not more than 4 nitrogen atoms per molecule.

7. A process according to claim 6 wherein the amine comprises at least one member selected from 1,2-diaminoethane, 1,3-diaminopropane, 1,4-diaminobutane, 1,6-diaminohexane, diethylene triamine, triethylene tetramine, 1,2-propylene diamine, di(1,2-propylene)triamine, di(1,3-propylene)triamine, N,N-dimethyl-1,3-diaminopropane, N,N-di-(2-aminoethyl)ethylene diamine, N,N-di(2-hydroxyethyl)-1,3-propylene diamine, 2-propyldodecylamine, N-dodecyl-1,3-propane diamine, diisoproanolamine, diethanolamine, and N-(3-aminopropyl)morpholine.

8. A process according to claim 1 wherein the amine comprises at least one polyoxyalkylene polyamine of the formulae:
NH₂-alkylene-(-O-alkylene-)ₘ-NH₂
where m has a value of 1 to 2, and
R-(-alkylene-[-O-alkylene-]ₙ-NH₂)ₐ
where n has a value of 1 to 2, R is a substituted saturated hydrocarbon radical of from 1 to 3 carbon atoms, wherein the number of substituents on the R group is represented by the value of "a" which is a number from 1 to 3.

9. A process according to claim 8 wherein said alkylene groups are straight or branched chain and contain from 2 to 4 carbon atoms.

10. A process according to any preceding claim wherein said amine and said product of step (a) are contacted with stirring at a temperature of from 100 to 150°C for a period from 30 min. to 3 hours.

11. A process according to any of claims 1 to 9 wherein said amine and said product of step (a) are contacted with stirring at a temperature of from 110 to 135°C for a period from 30 min. to 3 hours.

12. A process according to any preceding clain wherein from 1 to 10 equivalents of reactive primary or secondary amine are provided per mole of dicarboxylic acid moiety of the product of step (a).

13. A process according to any of claims 1 to 10 wherein from 1.5 to 5 equivalents of reactive primary or secondary amine are provided per mole of dicarboxylic acid moiety of the product of step (a).

14. A process according to any preceding claim wherein the liquid reaction solvent is a hydrocarbon oil.

15. A process according to claim 14 wherein step (a) is carried out in the presence of said hydrocarbon oil and the produced solution is passed to step (b).

16. A process according to any preceding claim wherein the liquid reaction solvent is a lubricating oil.

## Patentansprüche

1. Verfahren zur Herstellung einer ölhaltigen bzw. ölartigen Lösung mit verminderter Viskosität, die Kupfersalze polyolefinischer Dicarbonsäuren enthält, bestehend aus den Schritten:
(a) Herstellung eines Kupfersalzes eines polyolefinisch substituierten Dicarbonsäurematerials, wobei der polyolefinische Substituent, der ein Zahlenmittel des Molekulargewichts von mehr als 600 hat, sich von einem Olefinpolymer eines C₂- bis C₁₀-Monoolefins ableitet, und der Dicarbonsäureteil sich von einem einfach ungesättigten C₄- bis C₁₀-Dicarbonsäurematerial ableitet, und
(b) Reaktion oder Komplexierung mindestens eines Teils des Produkts aus Schritt (a) in einem flüssigen Reaktionslösungsmittel mit einem Amin, ausgewählt aus aliphatischen und cycloaliphatischen Aminen, das 1 bis 4 Stickstoffatome pro Molekül enthält, wobei das Amin mindestens ein primäres oder sekundäres Stickstoffatom pro Molekül hat.

2. Verfahren gemäß Anspruch 1, wobei das einfach ungesättigte Säurematerial mindestens einen Vertreter, ausgewählt aus Maleinsäure, Maleinsäureanhydrid, Itakonsäure, Chlormaleinsäure, Chlormaleinsäureanhydrid und Dimethylfumarat, enthält.

3. Verfahren gemäß Anspruch 1 oder Anspruch 2, wobei der poly-olefinsiche Substituent Polyisobutylen, Polybutylen oder Mischungen davon umfaßt.

4. Verfahren gemäß einem der vorhergehenden Ansprüche, wobei der polyolefinische Substituent sich von einem Polymer, das ein Zahlenmittel des Molekulargewichts von 900 bis 3000 hat, ableitet.

5. Verfahren gemäß Anspruch 4, wobei das polyolefinisch substituierte Dicarbonsäurematerial ausgewählt wird aus Polyisobutenyl- oder Polybutenylbernsteinsäure oder -anhydrid.

6. Verfahren gemäß einem der vorhergehenden Ansprüche, wobei das Amin mindestens ein aliphatisches, gesättigtes Amin mit den allgemeinen Formeln umfaßt: wobei R, R′, R˝ und R˝′ unabhängig aus Wasserstoff, geraden oder verzweigten C₁- bis C₂₅-Alkylketten, C₁- bis C₁₂-Alkoxy und C₂- bis C₆-Alkylen ausgewählt sind, und wobei R˝′ zusätzlich einen Teil mit der Formel: enthalten kann, wobei R′ wie oben definiert ist, und wobei s und s′ gleiche oder verschiedene Zahlen von 2 bis 6 sein können, und t und t′ gleiche oder verschiedene Zahlen zwischen 0 und 2 sein können, unter der Voraussetzung, daß das Amin nicht mehr als 4 Stickstoffatome pro Molekül enthält.

7. Verfahren gemäß Anspruch 6, wobei das Amin mindestens einen Vertreter umfaßt, der aus 1,2-Diaminoethan, 1,3-Diaminopropan, 1,4-Diaminobutan, 1,6-Diaminohexan, Diethylentriamin, Triethylentetramin, 1,2-Propylendiamin, Di(1,2-propylen)triamin, Di(1,3-propylen)triamin, N,N-Dimethyl-1,3-di-aminopropan, N,N-Di-(2-aminoethyl)ethylendiamin, N,N-Di(2-hydroxyethyl)-1,3-propylendiamin, 2-Propyldodecylamin, N-Dodecyl-1,3-propandiamin, Diisopropanolamin, Diethanolamin und N-(3-Aminopropyl)morpholin ausgewählt ist.

8. Verfahren gemäß Anspruch 1, wobei das Amin mindestens ein Polyoxyalkylenpolyamin der folgenden Formeln umfaßt:
NH₂-Alkylen-(-O-Alkylen-)ₘ-NH₂,
in der m einen Wert von 1 bis 2 hat, und
R-(-Alkylen-[-O-Alkylen-]ₙ-NH2)ₐ,
in der n einen Wert von 1 bis 2 hat, R ein substituierter, gesättigter Kohlenwasserstoffrest mit 1 bis 3 Kohlenstoffatomen ist wobei die Zahl der Substituenten an der Gruppe R durch den Wert "a" dargestellt wird, der eine Zahl von 1 bis 3 ist.

9. Verfahren gemäß Anspruch 8, wobei die Alkylengruppen gerad-oder verzweigtkettig sind und 2 bis 4 Kohlenstoffatome enthalten.

10. Verfahren gemäß einem der vorhergehenden Ansprüche, wobei das Amin und das Produkt aus Schritt (a) unter Rühren bei einer Temperatur von 100 bis 150°C während einer Dauer von 30 Minuten bis 3 Stunden kontaktbehandelt werden.

11. Verfahren gemäß einem der Ansprüche 1 bis 9, wobei das Amin und das Produkt aus Schritt (a) unter Rühren bei einer Temperatur von 110 bis 135°C während einer Dauer von 30 Minuten bis 3 Stunden kontaktbehandelt werden.

12. Verfahren gemäß einem der vorhergehenden Ansprüche, wobei zwischen 1 bis 10 Äquivalenten des reaktiven primären oder sekundären Amins pro Mol des Dicarbonsäureanteils des Produktes aus Schritt (a) eingesetzt werden.

13. Verfahren gemäß einem der Ansprüche 1 bis 10, wobei zwischen 1,5 bis 5 Äquivalenten des reaktiven primären oder sekundären Amins pro Mol des Dicarbonsäureanteils des Produktes aus Schritt (a) eingesetzt werden.

14. Verfahren gemäß einem der vorhergehenden Ansprüche, wobei das Reaktionslösungsmittel ein Kohlenwasserstofföl ist.

15. Verfahren gemäß Anspruch 14, wobei Schritt (a) in Gegenwart des Kohlenwasserstofföls ausgeführt wird, und die hergestellte Lösung Schritt (b) zugeführt wird.

16. Verfahren gemäß einem der vorhergehenden Ansprüche, wobei das Reaktionslösungsmittel ein Schmieröl ist.

## Revendications

1. Procédé de production d'une solution oléagineuse contenant des sels de cuivre d'acides dicarboxyliques polyoléfiniques ayant une viscosité réduite, qui comprend les étapes consistant :
(a) à prendre un sel de cuivre d'une matière acide dicarboxylique à substituant polyoléfinique, ledit substituant polyoléfinique étant dérivé d'un polymère oléfinique d'une mono-oléfine en C₂ à C₁₀ ayant une moyenne numérique du poids moléculaire supérieure à 600 et ledit groupement acide dicarboxylique étant dérivé d'une matière acide dicarboxylique mono-insaturée en C₄ à C₁₀ ; et
(b) à faire réagir ou à complexer au moins une portion du produit de l'étape (a) dans un solvant réactionnel liquide avec une amine choisie entre des amines aliphatiques et cycloaliphatiques contenant 1 à 4 atomes d'azote par molécule, ladite amine ayant au moins un atome d'azote primaire ou secondaire par molécule.

2. Procédé suivant la revendication 1, dans lequel la matière acide mono-insaturée comprend au moins un représentant choisi entre l'acide maléique, l'anhydride maléique, l'acide itaconique, l'acide chloromaléique, l'anhydride chloromaléique et le fumarate de diméthyle.

3. Procédé suivant la revendication 1 ou la revendication 2, dans lequel le substituant polyoléfinique comprend un polyisobutylène, un polybutylène ou leurs mélanges.

4. Procédé suivant l'une quelconque des revendications précédentes, dans lequel le substituant polyoléfinique est dérivé d'un polymère ayant une moyenne numérique du poids moléculaire de 900 à 3000.

5. Procédé suivant la revendication 4, dans lequel la matière acide dicarboxylique à substituant polyoléfinique est choisie entre un acide polyisobutényl- ou polybuténylsuccinique ou son anhydride.

6. Procédé suivant l'une quelconque des revendications précédentes, dans lequel l'amine comprend au moins une amine aliphatique saturée de formules générales : dans laquelle R, R′, R˝ et R˝′ sont choisis indépendamment entre l'hydrogène, des groupes alkyle à chaîne droite ou ramifiée en C₁ à C₂₅, un groupe alkoxy en C₁ à C₁₂ et un groupe alkylène en C₂ à C₆ et R˝′ peut en outre comprendre un groupement de formule dans laquelle R′ est tel que défini ci-dessus, et chacun des indices s et s′, qui peuvent être identiques ou différents, représente un nombre de 2 à 6, et t et t′, qui peuvent être identiques ou différents, représentent un nombre de 0 à 2, sous réserve que l'amine ne contienne pas plus de 4 atomes d'azote par molécule.

7. Procédé suivant la revendication 6, dans lequel l'amine comprend au moins un représentant choisi entre le 1,2-diaminoéthane ; le 1,3-diaminopropane ; le 1,4-diaminobutane ; le 1,6-diaminohexane ; la diéthylènetriamine ; la triéthylènetétramine ; la 1,2-propylènediamine ; la di-(1,2-propylène)triamine ; la di-(1,3-propylène)triamine ; le N,N-diméthyl-1,3-diaminopropane ; la N,N-di-(2-aminoéthyl)-éthylènediamine;la N,N-di-(2-hydroxyéthyl)-1,3-propylènediamine ; la 2-propyldodécylamine ; la N-dodécyl-1,3-propanediamine ; la diisopropanolamine ; la diéthanolamine et la N-(3-aminopropyl)morpholine.

8. Procédé suivant la revendication 1, dans lequel l'amine comprend au moins une polyoxyalkylènepolyamine de formules :
NH₂-alkylène-(-O-alkylène-)ₘ-NH₂
dans laquelle m a une valeur de 1 à 2, et
R-(-alkylène-[-O-alkylène-]ₙ-NH₂)ₐ
dans laquelle n a une valeur de 1 à 2, R est un radical hydrocarboné saturé substitué ayant 1 à 3 atomes de carbone, le nombre de substituants du groupe R étant représenté par la valeur de "a" qui est un nombre de 1 à 3.

9. Procédé suivant la revendication 8, dans lequel les groupes alkylène sont des groupes à chaîne droite ou ramifiée et contiennent 2 à 4 atomes de carbone.

10. Procédé suivant l'une quelconque des revendications précédentes, dans lequel l'amine et le produit de l'étape (a) sont maintenus en contact sous agitation à une température de 100 à 150°C pendant une période de 30 minutes à 3 heures.

11. Procédé suivant l'une quelconque des revendications 1 à 9, dans lequel l'amine et le produit de l'étape (a) sont maintenus en contact sous agitation à une température de 110 à 135°C pendant une période de 30 minutes à 3 heures.

12. Procédé suivant l'une quelconque des revendications précédentes, dans lequel on prévoit 1 à 10 équivalents d'amine primaire ou secondaire réactive par mole de groupement acide dicarboxylique du produit de l'étape (a).

13. Procédé suivant l'une quelconque des revendications 1 à 10, dans lequel on prévoit 1,5 à 5 équivalents d'amine réactive primaire ou secondaire par mole de groupement acide dicarboxylique du produit de l'étape (a).

14. Procédé suivant l'une quelconque des revendications précédentes, dans lequel le solvant réactionnel liquide est une huile hydrocarbonée.

15. Procédé suivant la revendication 14, dans lequel l'étape (a) est conduite en présence de ladite huile hydrocarbonée et la solution produite est transférée dans l'étape (b).

16. Procédé suivant l'une quelconque des revendications précédentes, dans lequel le solvant réactionnel liquide est une huile lubrifiante.
